

W. NERNST.  
ELECTRIC GLOW LAMP.  
APPLICATION FILED MAR. 29, 1898.

900,416.

Patented Oct. 6, 1908.



WITNESSES:

Chas. J. Clagett  
Wm. G. Lapey

INVENTOR

Walther Nernst.  
BY  
Charles A. Perry -  
ATTORNEY

# UNITED STATES PATENT OFFICE.

WALTHER NERNST, OF GÖTTINGEN, GERMANY, ASSIGNOR, BY MESNE ASSIGNMENTS, TO NERNST LAMP COMPANY, OF PITTSBURG, PENNSYLVANIA, A CORPORATION OF PENNSYLVANIA.

## ELECTRIC GLOW-LAMP.

No. 900,416.

Specification of Letters Patent.

Patented Oct. 6, 1908.

Application filed March 29, 1898. Serial No. 675,603.

*To all whom it may concern:*

Be it known that I, WALTHER NERNST, a subject of the German Emperor, residing at Göttingen, in the Kingdom of Prussia, German Empire, have invented certain new and useful Improvements in Electric Glow-Lamps, of which the following is a specification.

My invention relates to the class of electric lamps in which the light emitting element or member is a non-conductor at ordinary temperatures and which may be made conductive by subjecting it to a relatively high degree of heat.

15 The object of my invention is to provide a light emitting member or glower of such composition of materials as shall specially adapt it for efficient service and long life.

I have found that a glower formed of a mixture of certain materials will become conductive at a lower temperature and be more durable in service than a glower made of a single material, provided the materials are thoroughly powdered and mixed together, 25 then combined with a suitable binding material, and formed into the proper shape and thoroughly baked, suitable terminals of conducting material being attached to the ends of the glower in order to facilitate connecting 30 it in circuit for operation.

My invention contemplates the employment of any one of a considerable variety of mixtures of materials, but mixtures of two or more of the oxides of zirconium, yttrium, 35 thorium, beryllium, and magnesium will generally be found most desirable. I may, however, combine one of these oxides, such, for example, as the oxide of magnesium, with a small percentage of boric acid, chlorid of calcium, 40 tungstic acid, or the like.

When a glower formed of a proper mixture of two or more of the materials above specified is connected in an electric circuit and

heated to its conducting temperature, the heat developed in itself by the passage of a current therethrough will serve to maintain it in a conducting condition and cause it to yield light in a very efficient manner.

As an illustration of my invention, I show, in the accompanying drawing, a glower 1 which is a non-conductor at ordinary temperatures. As a simple means for raising the glower to conducting temperature, I show a torch 2 supported upon a suitable base 3.

It is to be understood that the illustration is in no sense restrictive, as regards either the form and dimensions of the glower or the means employed for heating it to conducting temperature.

I claim as my invention:

1. An improved glower for electrical incandescent lamps which is a non-conductor when cold but which becomes a good conductor and incandescent under the action of an electric current at high temperatures, and which consists essentially of a mixture of refractory metallic oxids.

2. An improved glower for electrical incandescent lamps which is a non-conductor at normal atmospheric temperatures but which readily becomes conductive and incandescent under the action of an electric current when heated, comprising a mixture of zirconium oxide and another refractory metallic oxide.

3. An improved glower for electrical incandescent lamps which is a non-conductor at normal atmospheric temperatures but which readily becomes conductive and incandescent under the action of an electric current when heated, comprising a mixture of zirconium oxide with thorium oxide.

Signed at Berlin this 17 day of March 1898.

WALTHER NERNST.

Witnesses:

CHAS. H. DAY,  
PAUL E. HUCHTNER.